

June 5, 1928.

1,672,172

W. REUSS

METHOD OF ANNEALING SHEET METAL

Filed June 24, 1926

*Fig. 1.*



*Fig. 2.*



Inventor:  
Wilhelm Reuss.  
by:  
Watson, Cott, Morse & Grindley.  
Attorney.

Patented June 5, 1928.

1,672,172

# UNITED STATES PATENT OFFICE.

WILHELM REUSS, OF ALTENA, GERMANY, ASSIGNOR TO JOH. MORITZ RUMP A.-G., OF ALTENA, GERMANY, A JOINT STOCK COMPANY OF GERMANY.

## METHOD OF ANNEALING SHEET METAL.

Application filed June 24, 1926, Serial No. 118,334, and in Germany September 25, 1925.

My invention relates to improvements in the method of annealing sheet metal. In the manufacture of the receivers used in telephony and radio, industry the diaphragms 5 must be made from perfectly plane sheet metal which is free of tension. When annealing a pile of superposed plates, as is usual for example in the manufacture of fine sheet metal, it is impossible completely to 10 remove the uneven parts of the blanks resulting from cold rolling and cutting. When wrapping the pile of plates in sheet metal and annealing the same under pressure and between plane plates the sheet 15 metal strips are frequently welded together by the gravity of the superposed piles and iron plates. Further, the wrapping of the piles of sheet metal requires much time and is expensive. The object of the improvements 20 is to provide a method by means of which the irregularities of the surface of the sheet metal are removed, in which there is no welding of the sheet metal plates, and which can be carried out at low cost. With 25 this object in view my invention consists in separating the piles of sheet metal strips by parallel members made from a material having a coefficient of expansion different from that of the sheet metal, and annealing the 30 piles under pressure.

In carrying out my improved method I pack the sheet metal strips within a rectangular annealing casing so that the individual plates are disposed vertically and fill out 35 the breadth of the casing, the casing being made from a material having a coefficient of expansion lower than that of the blanks. For example, when annealing sheet metal strips made from iron having a coefficient of 40 expansion of about 0.000011 I use an annealing box made from an iron-nickel alloy containing about 36% of nickel, said alloy being known in the trade under the name of invar and having a coefficient of expansion of 45 about 0.00000045. When heating the sheet metal strips at annealing temperature which in case of iron is from 400 to 600° C. the expansion of the sheet metal exceeds that of the box, so that the small interstices between 50 the successive metal strips resulting from packing the piles are removed. The plates are forced against the walls of the annealing box, and the irregularities resulting from cold rolling are perfectly removed.

55 Preferably plane plates made from a mate-

rial having a coefficient of expansion higher than that of the metal strips are placed at suitable distance apart between the sheet metal strips, in which case the smoothing action may be increased by applying higher pressure to the pile. For example, when annealing iron strips I use copper plates having a coefficient of expansion of 0.000017. 60

In order that my invention be more clearly understood a pile of metal plates packed in an annealing box has been shown in the accompanying drawing, in which

Fig. 1, is a sectional elevation of the pile and box and

Fig. 2, is a top plan view of Fig. 1. 70

As appears from the figures, the sheet metal strips *b* are vertically disposed within an annealing box *a* so as to fill out the whole breadth of the rectangular annealing box. The box *a* is made from a material having a 75 low coefficient of expansion, such for example as invar. Between the piles of sheet metal strips there are spaced plates *c* made from a material having a coefficient of expansion higher than that of the strips to be 80 annealed. The box is heated at the desired temperature say from 400 to 600° C. within an annealing furnace, and thereafter it is slowly cooled. After removing the strips from the box the sheet metal plates are found 85 to be perfectly plane and free of tension.

While in describing the invention reference has been made to sheet metal used in the manufacture of telephoned diaphragms and the like I wish it to be understood that 90 my improved method may be generally used for annealing sheet metal wherever a sheet metal is needed which is perfectly smooth and free of tension. For example I may use the method for annealing sheet metal 95 used in the manufacture of cases for photographic apparatus.

I claim:

1. The method of annealing sheet metal, which consists in subjecting a pile of parallel plates of sheet metal to a pressure which varies in proportion to the temperature to which the metal is subjected, by heating the plates and at the same time restraining the outer surfaces of the outermost plates equally throughout their entire area to resist the expansion in thickness of the plates during heat treatment, whereby the gradual expansion of the material due to increase of temperature resisted by the restraining effect 110

will generate a gradually increasing pressure to remove irregularities in the sheet material being annealed.

2. The method of annealing sheet metal, 5 which consists in subjecting a pile of parallel plates of sheet metal to a pressure which varies in proportion to the temperature to which the metal is subjected, by interspersing among the plates of the pile, other 10 plates of a material having a greater coefficient of expansion and heating the plates while restraining the outer surfaces of the outermost plates, whereby the combined expansion in thickness of the plates of the pile 15 and the interspersed plates as the temperature is increased will generate a gradually increasing pressure to remove irregularities in the sheet metal being annealed.

3. The method of annealing sheet metal, 20 which consists in subjecting the metal to a pressure during heat treatment which varies in proportion to the temperature thereof, by placing a pile of parallel plates of the sheet metal snugly between abutments having 25 a coefficient of expansion smaller than that of the metal, and which are substantially co-extensive in area with the adjacent surfaces of the outer plates and then heating

the plates, whereby the gradual expansion in thickness of the plates due to the increase 30 in temperature, resisted by the abutments will generate a gradually increasing pressure to remove irregularities in the sheet metal being annealed.

4. The method of annealing sheet metal, 35 which consists in subjecting the metal to a pressure during heat treatment which varies in proportion to the temperature thereof, by placing a pile of parallel plates of the sheet metal snugly in a container having a coefficient of expansion smaller than that of the metal, with the plates vertical to avoid the effect of their weight, and the outer plates of the pile abutting the two opposite walls 40 of the container, and the intermediate plates 45 being in contact with each other and then heating the plates whereby the gradual expansion in thickness of the plates due to increase of temperature resisted by the abutment will generate a gradually increasing pressure to remove irregularities in the sheet metal being annealed.

In testimony whereof I hereunto affix my signature.

WILHELM REUSS.